

## UNITED STATES PATENT OFFICE

WILLIAM S. CALCOTT, OF PENNS GROVE, NEW JERSEY, AND HERBERT W. WALKER, OF WILMINGTON, DELAWARE, ASSIGNORS TO E. I. DU PONT DE NEMOURS & COMPANY, OF WILMINGTON, DELAWARE, A CORPORATION OF DELAWARE

## NONCORROSIONAL ALCOHOLIC SOLUTION

No Drawing.

Application filed September 11, 1928. Serial No. 305,319.

This invention relates to the preparation of aqueous alcoholic solutions which are substantially inert with respect to iron. More particularly it pertains to the use of alkyl and alkylol amines as a class of compounds which act as inhibitors for iron corrosion by aqueous solutions of mono and polyhydric alcohols.

It is well known that water solutions of alcohols attack metallic iron very rapidly under ordinary conditions and considerable corrosion as manifested by rust spots, deposits, and sediment takes place.

We have found that if a small amount of an alkyl amine, such as, di-n-propylamine iso propylamine, di-butyl amine, or iso amylamine, be added to a mono or polyhydric alcohol and the alcohol then diluted with water to any desired concentration there results a solution in which iron does not readily corrode. The presence of one of these amines prevents the iron from rusting and the metal remains bright, lustrous and free from scale and rust deposits. The alkyl amines have the general formula



Likewise, we have found that if a small amount of an ethanol amine, such as mono, di, or triethanol amine or mixtures of any two or all three in any proportion, be added to a mono- or polyhydric alcohol and the alcohol then diluted with water to any desired concentration, there results a solution in which the rate of corrosion of the iron is much less than in a solution not so treated with ethanol amines. A distinct protective action on iron is observed in alcohol solutions treated with these ethanol amines after heating several hours at 85-90°. In place of the ethanol amines a water soluble alkylol amine such as methanol amine or propanol amine may be employed. The alkylol amines have the general formula



where  $R_1$  and  $R_2$  represent either hydrogen or an alkyl or hydroxy-alkyl radical.

For purposes of illustration the following examples are furnished.

*Example 1.*—If di-butylamine in an amount sufficient to make 0.1% of the final solution be added to methyl alcohol, ethyl alcohol, glycerine or glycol and water added to the alcoholic solution of the amine to produce a 40% solution of alcohol there is thereby formed a solution which effectively inhibits the corrosion of iron ordinarily taking place in these solutions.

*Example 2.*—If diethanol amine or a mixture of 80% triethanolamine and 20% diethanol amine in an amount sufficient to make 0.1% of the final water solution be added to ethyl alcohol, glycerine or glycol and water added to the alcoholic solution of the amine to produce a 40% solution of alcohol there is thereby formed a solution which effectively inhibits the corrosion of iron ordinarily taking place in these solutions.

With the high boiling amines the property of inhibiting corrosion is retained at elevated temperatures, for example, at the boiling point of water. Such amines can therefore be advantageously employed to prevent corrosion of automobile radiators by mono and polyhydric alcohol anti-freeze mixtures, as well as storage tanks, drums, and cans composed of iron.

It will be understood that the alkyl amines, alkylol amines and alcohols named above are given by way of illustration only, and that it is not applicants' intention to be limited except as indicated by the scope of the appended claims.

Also, it will be understood that the amines may be used either singly or in combination, and may be employed to inhibit corrosion by a mixture of alcohols as well as to inhibit corrosion by individual alcohols.

We claim:

1. A process for minimizing the corrosion of iron by an aqueous alcoholic solution in contact therewith, which comprises contacting said solution with iron in the presence of a water soluble amine of the group consisting of alkyl and alkylol amines.

2. A process for minimizing the corrosion of iron by an aqueous alcoholic solution in

contact therewith, which comprises contacting said solution with iron in the presence of an amine of the group consisting of di-n-propylamine, iso-propylamine, di-butylamine, iso-amylamine, and the mono, di and triethanolamines.

3. A process for minimizing the corrosion of iron in the presence of an aqueous solution of an alcohol of the group consisting of 10 methyl and ethyl alcohols, glycerine and glycol, which comprises contacting said solution with iron in the presence of a water soluble amine of the group consisting of alkyl and alkylol amines.

15 4. A process for minimizing the corrosion of iron by an aqueous alcoholic solution, which comprises contacting said solution with iron in the presence of a water soluble alkylol amine.

20 5. A process for inhibiting the corrosion of iron by an aqueous alcoholic solution in contact therewith, which comprises contacting said solution with iron in the presence of an ethanol amine.

25 6. A process for inhibiting the corrosion of iron by an aqueous alcoholic solution in contact therewith, which comprises contacting said solution with iron in the presence of tri-ethanol amine.

30 7. A process for inhibiting the corrosion of iron by an aqueous alcoholic solution, which comprises contacting said solution with iron in the presence of a mixture of di- and tri-ethanol amines.

35 8. A non-corrosive mixture comprising an alcohol and an amine of the group consisting of di-n-propylamine, iso-propylamine, di-butylamine, iso-amylamine and the mono, di and tri-ethanol amines.

40 9. A non-corrosive mixture comprising an aqueous solution of an alcohol of the group consisting of methyl and ethyl alcohols, glycerine and glycol and tri-ethanol amine.

45 10. A non-corrosive mixture comprising an alcohol and a mixture of di- and tri-ethanol amines.

In testimony whereof we affix our signatures.

WILLIAM S. CALCOTT.  
HERBERT W. WALKER.